

# UNITED STATES PATENT OFFICE.

OSCAR EMIL WALTER STÖHRER, OF CHARLOTTENBURG, GERMANY.

## PROCESS OF MANUFACTURING NITROGLYCERIN EXPLOSIVES OF REDUCED FREEZING-POINT.

No. 855,595.

Specification of Letters Patent.

Patented June 4, 1907.

Application filed April 10, 1906. Serial No. 310,997.

*To all whom it may concern:*

Be it known that I, OSCAR EMIL WALTER STÖHRER, a subject of Prussia, residing at Charlottenburg, Germany, have invented a new and useful Process of Manufacturing Nitroglycerin Explosives of Reduced Freezing-Point, of which the following is a specification.

This invention relates to a process of transforming glycerin into diglycerin by means of simply heating the glycerin without additions. To this purpose, it will be advantageous to proceed as follows:—The glycerin is heated, under ordinary pressure and without any addition for some length of time until it boils vigorously (about 190° to 195° centigrade), there being used for this purpose a refrigerating condenser which allows the water formed during said process to distil over and the glycerin vapors to condense. If the heating operation is interrupted after 5 or 6 hours, there has formed in the viscous mass 55-65% diglycerin which can be obtained by distilling under a pressure of 8-10 mm., between 245°-250° centigrade as a very viscous liquid which is clear as water, and which tastes like glycerin, very sweet and absorbs water readily in the atmosphere. Molecular weights ascertained according to the method of lowering the freezing point, were in accordance with the theory (166). If one part of the diglycerin is gradually poured into ten parts of a mixture of 13 parts of water, 58 parts of sulfuric acid and 29 parts of nitric acid, at a temperature of 10-15 degrees C., there will be obtained, after repeated washing with water, a viscous slightly yellow colored liquid which is insoluble in water, but readily soluble in the usual organic solvents for example ether, alcohol, acetone, benzol and chloroform. The quantity of nitrogen contained in this liquid, of which it has been found that it amounts to 15.98%, confirms the formula  $C_6H_{10}(NO_3)_4O$ . The molecular weight was 331,—theory 346. The specific weight was 1.544. When exposed during several days to a temperature of -20° C., it does not show any inclination to freeze. When mixed with silicious sinter in proportion of 25 parts of silicious sinter to 75 parts of tetranitrodiglycerin and if shot in Trauzl's lead block

under the testing condition for guhr dynamite, there resulted an extension of 348 ccm. (nitroglycerin, if shot under the same condition, effects an extension of 398 ccm.). It can be made to crystallize only with the greatest difficulty and it congeals with much more difficulty than nitroglycerin and, if added to the latter, it acts in such a manner, that the latter, too, is rendered less congealable. A mixture of tetranitrodiglycerin and nitroglycerin in the proportion of 25 to 75 does not become frozen when exposed during a longer time at a temperature of -15 to -20 centigrade.

Mixtures which are so difficult to congeal can be obtained not only by means of adding tetranitrodiglycerin to nitroglycerin but also by means of nitrating a mixture of glycerin and diglycerin which may be obtained in the described manner, by means of heating glycerin. The method of making these mixtures is as follows:—Glycerin is heated under the conditions mentioned above and kept boiling until a sample taken after fractionation *in vacuo* shows a percentage of 75% glycerin and 25% diglycerin. This mixture is transformed into the nitrated product in the same manner as above described for the pure diglycerin and this product purified by washing with water and a solution of sodium carbonate and stabilized. The resulting stuff is an explosive oil, which possesses regarding the nitroglycerin the advantages mentioned above and can be worked up in the same manner to explosives and powders as nitroglycerin.

I claim:—

The process of preparing a mixture of tetranitrodiglycerin and trinitroglycerin consisting in heating glycerin to its boiling point under normal atmospheric pressure, maintaining the mass at boiling temperature until it contains the desired percentage of diglycerin and nitrating the resultant mixture, substantially as described.

In testimony whereof I have signed my name to this specification in the presence of two subscribing witnesses.

OSCAR EMIL WALTER STÖHRER.

Witnesses:

HENRY HASPER,  
WOLDEMAR HAUPT.